

May 31, 1927.

L. A. WYND ET AL

1,630,507

PROCESS OF COATING MATERIALS HAVING AN IRON OR STEEL BASE

Filed Feb. 26, 1926



INVENTORS.

Leo A. Wynd,  
Julian L. Schuler  
Charles A. Dake

ATTY

## UNITED STATES PATENT OFFICE.

LEO A. WYND AND JULIAN L. SCHUELER, OF PEORIA, ILLINOIS.

## PROCESS OF COATING MATERIALS HAVING AN IRON OR STEEL BASE.

Application filed February 26, 1926. Serial No. 90,868.

This invention has reference to a process of coating materials having an iron or steel base such as sheets, wires and like materials, particularly the coating of wire used in the fence industry and for telephone and other purposes.

The principal object of this invention is to apply a heavy coating of zinc on wire without recourse to heat-treatment, either prior to or after coating, or the use of a high grade zinc. Such a coating may be bent around its own diameter without showing the least signs of cracking or flaking and the coating will be smooth.

15 The invention has for a further object to permit higher speeds to be used for the formation of a heavier coating than can be economically done by any other process of which we have any knowledge.

20 The invention has for a further object an improved cleaning process for the wire prior to its entrance to the zinc bath and to allow the clean wire to enter and leave the bath through a clean zinc system.

25 Galvanized wire which is to be used for fabricating purposes, and more particularly that which is to be used in the manufacture of woven wire fencing, should have a relatively heavy coating of zinc in order to be able to withstand atmospheric rusting and 30 corroding conditions, and prior to our invention, so far as we are aware, this was not possible, except at an increased cost of production.

35 The universal practice for testing the relative value of zinc on galvanized wire is by the so-called Preece or copper sulphate test. There are other tests, however, which are used for quantitatively determining the 40 amount of spelter on galvanized wire, such as dipping the coating in caustic solution; in a suitable hydrochloric acid solution; in a solution of hydrochloric acid and antimony chloride, and in a lead acetate solution. The 45 copper sulphate test, although not quantitative, is comparable when used under known conditions of temperature and strength and being a quick test, and one which can be performed by anyone after a little experience, has come to be the routine testing medium for galvanized wire coating. On the basis of such tests as these, are determined the relative weights of coatings (either thin or heavy) referred to throughout this description.

55 At the present time, so far as we are

aware, there are only three methods in use whereby these heavy zinc coatings may be obtained by the hot process of galvanizing. The first method is to pass the wire through finely divided charcoal as it emerges from the galvanizing bath. By such a process a relatively smooth coating may be obtained. This method is principally used for making telephone and telegraph wire. It has serious drawbacks, however, from an economic standpoint because the wire must travel at a very slow speed and a very high grade zinc must be used and, furthermore, the coated wire cannot be subjected to the action of fence fabricating machines without the coating cracking or flaking-off of the iron base. The second method is to cause the wire to travel at a relatively slow speed through a zinc bath, the speed depending upon the gauge of the wire, the thickness of the coating desired and the length of the bath and then smoothing the coating by passing it between suitable wipes. This method, too, has its economic drawbacks because it requires pure zinc on account of the slow speeds required and it consequently lessens the tonnage passing through a galvanized unit in a given time. The third method is to pass the wire through a galvanizing bath and then without wiping subject it to a heat-treatment. This process, too, is slower than our process and more expensive to operate.

Therefore, by the use of our invention we are not only permitted to use higher speeds for galvanizing wire but we, also, obviate the necessity of using wipes or other smoothing mediums and the necessity for heat-treatment, either one or the other, heretofore considered indispensable in galvanizing operations. An advantage in eliminating the wipes is that a heavier coating is permitted to remain on the wire, which in ordinary processes is removed by the wipe as the coated wires pass therethrough. It will, therefore, be apparent to those skilled in the art that the higher speed can be used because it is not necessary for the wire to be wiped nor to be immersed in a molten salt bath, nor is it necessary to pass the coated wire through a heat-treating furnace. By the elimination of all three of these steps we considerably reduce cost and increase production, as will be apparent to those skilled in the art.

That the process herein described may be better understood, reference is had to the

accompanying drawing, in which a diagrammatic view illustrates a continuous galvanizing or coating apparatus, including a lead annealing bath; an acid bath, and a galvanizing tank adapted to contain the molten zinc bath. There is eliminated from such an apparatus the usual and ordinary wiping or smoothing mechanism, as well as a heat-treating furnace used for heat-treating the coating subsequent to the coating operation; also, there is eliminated the necessity for giving the wire a so-called preliminary carbonization before it enters the coating bath.

Our process is very simple. We have discovered that if a wire is given a very thorough cleaning prior to coating and if the wire is kept clean until and while it enters the coating bath and also kept clean as it leaves the coating bath and the coated wire is removed from the bath in a substantially vertical direction, that a very smooth coating will be obtained and a very heavy one at the same time, which can be subjected to the most severe bending or forming operations and still leave the coating intact upon the wire.

The processes which are at present in ordinary use, and which we are about to describe, have special reference to the lower carbon wires, though not limited to these, are used for fabricating fencing, barb wire, and for the manufacture of telephone wire and the like.

The ordinary process of galvanizing wire consists in passing the wire through molten lead or through an annealing furnace which accomplishes the same purpose, cooling the wire and then passing it into preferably muriatic acid where it is subjected to a cleaning operation. It passes from the muriatic acid through a flux, then over a drier and into the coating bath. As the wire leaves the bath it passes between asbestos wiping means of some kind—either pressure or lever wipes and these wipes remove the excess zinc; in some cases as much as 50% of the coating which adheres to the wire. This leaves a very thin coating on the wire.

In the manufacture of telephone wire, which requires a heavy coating, the wire is passed very slowly through a bath of high grade zinc and as it leaves the bath the wire passes through a bed of charcoal and tallow, which wipes and smoothes the coating but does not wipe it as heavily as the pressure wipes mentioned before. In the Herman process, United States Letters Patent No. 1,430,648, the wire passes through the coating bath and as it emerges from the bath the wire passes over a skimming arrangement which does not materially remove any coating, other than removing the dross and skimmings carried over, and then passes into a furnace where the heat-treatment, to which the wire is subjected, smoothes the coating

and makes it malleable and flexible. Another method for applying a heavy coating to wire is the method where the wire is subjected to a so-called preliminary carbonization before it enters the coating bath. This preliminary treatment may take place in a molten bath of some salt, or some combination of molten salts, and is claimed to allow a heavy coating to be carried on the wire which will be flexible. However, by this method it is also necessary to pass the wire through a wiping arrangement of some kind.

By our process the wire after being subjected to the usual annealing is passed into a usual cleaning solution, where it is subjected to a heavy current, approximately 110 volts D. C., the wire being in contact with the positive side of the current and a sheet of lead or some other suitable material being connected to the negative side of the current. This current drives any foreign matter off of the wire and leaves the wires extremely clean, especially from the action of the cleaning solution, which is extremely vigorous and activated when the current is passed through it. The wire then passes directly from the cleaning solution into the coating bath.

The wire enters the coating bath through a clean zinc surface and after passing through the zinc emerges from the bath through a similarly clean zinc surface. The wire leaves the bath without passing through any wiping, skimming or smoothing means of any kind and is conducted in substantially a vertical direction after leaving the bath until the coating has set, after which the direction of the wire may be as desired.

No other process is known to us whereby a heavy coating of "prime western zinc" may be applied to wire, and which is flexible, malleable and smooth, except the Herman process, United States Letters Patent No. 1,430,648, hereinbefore mentioned. "Prime western zinc" is the usual zinc used for coating wire, except in cases where a heavy coating is desired, such as for telephone or telegraph wire, where the coating is required to stand a bend around a mandrel twelve times the diameter of the wire, in which case recourse must be had to the use of a very high grade zinc such, for example, as pure electrolytic zinc or the equivalent thereof. The difference between the high grade zinc and the "prime western zinc" is, of course, well known and understood by those skilled in the art. By the ordinary processes of applying such coatings "prime western zinc" will not stand this bend test, as the coating will crack and peel off the wire upon subjecting it to the slightest amount of bending.

The bending properties of wire coated by our process are remarkable in that the coated wire may be wrapped around its own diameter, then unwrapped and again wrapped

around its own diameter without apparently affecting the coating in any manner. There is no other process known to us of any kind whereby this may be done with a heavy 5 "prime western zinc" coating.

In order to keep the surface of the wire clean at the entrance and exit ends of the coating bath, we apply small amounts of salammoniac or some other suitable material 10 at suitable intervals in order to keep foreign matter removed from said surface.

We are aware that the method of cleaning per se is not new, nor is the addition of salammoniac to zinc baths new, nor is 15 the removal of the wire from the zinc bath in substantially a vertical direction new, but the process as described by us, we believe, is new and produces results heretofore considered impossible with a coating 20 of "prime western zinc", and which could be produced with a very high grade zinc only under very carefully controlled conditions, which are far more expensive to operate than our process.

25 Our process is the cheapest one known to us for producing heavy zinc coatings, and more tonnage per coating unit can be obtained than by any other process known to us for producing heavy coatings of zinc 30 on wire.

The diagrammatic view accompanying this description shows a preferred form of apparatus by means of which the within described process may be practiced, and is 35 offered to show a mode of application in which an annealing furnace 1, a cleaning bath 2 and a coating tank 3 are placed in substantially the relative positions they will occupy when employing the process. A wire 40 A is shown threading through in the act of being coated.

At the entrance end of the cleaning bath there is illustrated a positive contact 4 with which the wire A engages, and within the 45 cleaning bath 2 there is provided a negative connection 5, which may be preferably a lead sheet, arranged across the bottom of the cleaning bath and within the cleaning solution. These elements 4 and 5, as, of course, 50 will be understood, are connected in a suitable manner to a source of electric supply not shown.

The coating tank 3 is provided at its entrance end with a compartment 8 and its 55 exit end a similar compartment 9. These compartments are both formed by means of aprons 10. Above the compartments 8 and 9 are arranged feeding receptacles 6 and 7 respectively, containing suitable mechanisms, not shown, by means of which a suitable amount of salammoniac may be added at suitable intervals to compartments 8 and 9 respectively.

The amount of salammoniac added, and 60 the intervals at which it is added, depends

on the size of the coating bath, the gauge of the wire passing therethrough and the rate of speed at which said wire is traveling, but in any case the amount added is very small.

In substance, our process consists in producing a heavy, flexible and malleable coating of "prime western zinc" on wire without recourse to a heat-treating process and in which we eliminate the usual wiping or 70 smoothing or skimming mechanisms, or heat-treating apparatus for the coating. It is obvious, of course, that as we produce such a coating, as has been described, using "prime western zinc" that we can readily do 75 so using a high grade zinc.

The coating which is formed on the wire by our process, using "prime western zinc", is extremely malleable and flexible and has a very bright silvery color, which it retains 80 for a long period of time. This coating has properties heretofore considered impossible to obtain with "prime western zinc", and which prior to our invention has been impossible to duplicate by any process known 85 to us.

It is true, of course, that the heat-treating process of Herman, United States Letters Patent No. 1,430,648, produces a malleable coating using "prime western zinc" but 90 it is not as malleable or flexible as the coating produced by our process and we have eliminated the necessity for heat-treating 95 the coating.

The terms and expressions which we have 100 employed are used as terms of description and not of limitation and we have no intention in the use of such terms and expressions of excluding any equivalent for the features shown and described, and recognize 105 that various modifications are possible within the scope of the invention claimed.

This application is a companion to the application filed by applicants on March 20, 1926, for a galvanizing apparatus bearing Serial No. 96,301.

What we claim is:—

1. A process for applying smooth zinc coatings to iron or steel wire, independent of wiping, which consists in subjecting the wire 115 to an activated cleaning prior to its entrance to a coating bath, passing the wire thru the coating bath, the entrance of the wire and the exit of the wire from the coating bath being through substantially clean zinc surfaces.

2. A process for applying smooth zinc coatings to iron or steel wire, which consists in subjecting the wire to an activated cleaning prior to its entrance to a coating bath, passing the wire thru the coating bath, the entrance of the wire and the exit of the wire from the coating bath being through substantially clean zinc surfaces, and conducting the wire from the bath in substantially 125 130

- a vertical direction whereby wiping is obviated.
3. A process for applying heavy flexible, malleable and smooth coatings of zinc to iron or steel wire independent of wiping, which consists in subjecting the wire to an activated cleaning prior to its entrance to a coating bath, passing the wire thru the coating bath, the entrance of the wire and the 10 exit of the wire from the coated bath being through substantially clean zinc surfaces.
4. A process for applying heavy, flexible, malleable and smooth coatings of zinc to iron or steel wire, which consists in subject- 15 ing the wire to an activated cleaning prior to its entrance to a coating bath, passing the wire thru the coating bath, the entrance of the wire and the exit of the wire from the coated bath being through substantially 20 clean zinc surfaces, and conducting the wire from the bath in substantially a vertical direction whereby wiping is obviated.
5. A process for applying heavy, flexible, malleable and smooth coatings of "prime western zinc" to iron or steel wire, independent of wiping, which consists in subjecting the wire to an activated cleaning prior to its entrance to a coating bath, pass- 25
- ing the wire thru the coating bath, the entrance of the wire and the exit of the wire from the coated bath being through substantially 30 clean zinc surfaces.
6. A process for applying heavy, flexible, malleable and smooth coatings of "prime western zinc" to iron or steel wire, which consists in subjecting the wire to an activated cleaning prior to its entrance to a coating bath, passing the wire thru the coating bath, the entrance of the wire and the 35 exit of the wire from the coated bath being through substantially clean zinc surfaces, and conducting the wire from the bath in substantially a vertical direction whereby 40 wiping is obviated.
7. A process for applying smooth zinc 45 coatings to iron or steel material, independent of wiping, which consists in subjecting the material to an activated cleaning prior to its entrance to a coating bath, passing the material thru the coating bath, the entrance of the material and the exit of the material 50 from the coating bath being thru substantially clean zinc surface.

LEO A. WYND.  
JULIAN L. SCHUELER.